# EUROPEAN PATENT SPECIFICATION

(11) **EP 1 964 969 B1**
(45) Date of publication and mention of the grant of the patent: **11.07.2018**
(21) Application number: 08152014.0
(22) Date of filing: 27.02.2008
(51) Int. Cl.: D21H 19/54, D21H 17/28, D21H 21/18

(54) **COATING COMPOSITIONS**
BESCHICHTUNGSZUSAMMENSETZUNGEN
COMPOSITION DE REVETEMENT

(30) Priority: 27.02.2007 EP 07103158
(43) Date of publication of application: 03.09.2008
(73) Proprietor: Cargill, Incorporated, Wayzata, MN 55391 (US)
(72) Inventor: Berckmans, Marc Charles Florent, 1030, Bruxelles (BE); Glittenberg, Detlev, D-47807, Krefeld (DE); Roux, Rudy, 59500, Douai (FR)
(74) Representative: Wilkinson, Stephen John

(56) References cited:
- EP-A- 0 278 582
- EP-A2- 0 319 989
- EP-A2- 0 374 993
- WO-A-2005/052255
- GB-A- 602 223
- GB-A- 871 937
- US-A- 2 849 326
- US-B1- 6 265 570

## Description

### Technical Field of the Invention

The present invention relates to coating compositions and, in particular, to paper coating compositions containing specific starchy materials.

### Background of the Invention

Coating compositions are used on a number of substrates including, amongst others, metals, plastics, textiles and paper. They help to protect and enhance the feel and appearance of the surfaces to which they are applied. They may also improve other characteristics such as printability, water resistance, reflectivity or strength.

The make up of a coating composition will depend on its desired end-use. Typically, a paper coating composition (also known as a "coating colour") will contain pigments, binders and thickeners.

Thickeners, in particular, have to be chosen very carefully as they are responsible for determining the coating composition's rheological properties (both at high and low shear) and will contribute to it having an appropriate stability (e.g. during storage or at the high temperatures required for drying). To this end, a number of starch products have been developed. The aim of these developments has been the production of a cheap, highly stable, highly viscous, cold water soluble starch.

Cold water solubility is indeed considered important if surface graininess is to be avoided. It can also ease application of the coating composition and generally improve the overall characteristics of the finished product. A lot of research has therefore gone into finding new ways of increasing the cold water solubility of starch thickeners. US6191116 (National Starch), for example, describes a process for obtaining 100% cold water soluble starch derivatives suitable for use in coating compositions. The process involves dehydrating a starch substrate and then dextrinising it under anhydrous conditions.

US2849326 relates to a composition and method of preparation of pigments coating containing high solids content for paper and polymers derived from starch.

GB602223 relates to the manufacturing of cold-water soluble and cold-water swelling starches and their use in sand cores, as odour binders and for coating and sizing of paper, textiles and the like.

Unfortunately, despite all these efforts, the cold water soluble starches currently being used in the industry still have a number of drawbacks, the most important one being cost. Conventional cold water soluble starches are prepared by gelatinisation in the presence of water followed by drying. The drying step is expensive in terms of both time and energy. The resulting high costs limit the use of these starches to higher added value coating applications.

It is therefore apparent that there is a need in the art for a new cold water soluble starch which can be used at high concentrations in coating compositions without prohibitively increasing their cost. The present invention provides such a starch.

### Summary of the Invention

A coating composition comprising a cold water soluble starch and one or more binders, thickeners and/or pigments characterized in that said cold water soluble starch is derived from a starch selected from the group consisting of wheat starch, corn starch and mixtures thereof, and has a DE of less than 5 and has :
- a number of average molecular weight (Mn) of 3500 to 20000 Daltons;
- a granular structure before solubilisation;
- a solubility at pH and 20°C (S1) of 30 to 90%; and
- a solubility at pH10 and 35°C (S2) which is at least 10% greater than S1.

In a further aspect of the present invention, there is provided a paper coating composition as defined above.

In a yet further aspect of the present invention, there is provided a paper product coated with the above coating composition.

In a final aspect of the present invention, there is provided the use of a cold water soluble starch as defined above for the production of a coating composition.

### Brief Description of the Figures

Figure 1 - compares water release properties of a standard precoat composition and a precoat composition of the present invention.
Figure 2 - compares the paper gloss levels of a paper product coated with a standard precoat composition and with a precoat composition of the present invention.
Figure 3 - compares the printing gloss levels of a paper product coated with a standard precoat composition and with a precoat composition of the present invention.
Figure 4 - compares the pick-dry properties of a paper product coated with a standard precoat composition and with a precoat composition of the present invention.
Figure 5 - compares water release properties of a standard topcoat composition and a topcoat composition of the present invention.
Figure 6 - compares the paper gloss levels of a paper product coated with a standard topcoat composition and with a topcoat composition of the present invention.
Figure 7 - compares the printing gloss levels of a paper product coated with a standard topcoat composition and with a topcoat composition of the present invention.
Figure 8 - compares the mottling levels of a paper product coated with a standard topcoat composition and with a topcoat composition of the present invention.
Figure 9 - compares levels of coating cracking for a paper product coated with a standard topcoat composition and with a topcoat composition of the present invention.

### Detailed Description of the Invention

A coating composition comprising a cold water soluble starch and one or more binders, thickeners and/or pigments characterized in that said cold water soluble starch is derived from a starch selected from the group consisting of wheat starch, corn starch and mixtures thereof, and has a DE of less than 5 and has :
- a number of average molecular weight (Mn) of 3500 to 20000 Daltons;
- a granular structure before solubilisation;
- a solubility at pH and 20°C (S1) of 30 to 90%; and
- a solubility at pH10 and 35°C (S2) which is at least 10% greater than S1.

The CWSS is derived from a starch selected from the group consisting of: corn starch, wheat starch, and mixtures thereof.

The expression "modified starch" as used herein refers to a starch whose structure has been altered by chemical, enzymatic or heat treatment. For instance, the starch substrate may be selected from esterified, etherified, cross-linked, oxidised or acid modified starches or mixtures of two or more thereof. The CWSS of the invention is not be strongly degraded; in other words, it has a dextrose equivalence (DE) value of less than 5, more preferably of less than 4, more preferably of less than 3, more preferably of less than 2 (wherein DE is measured using the Schoorl Method).

Before solubilisation, the CWSS of the present invention will have a granular structure. Native starch granules exist in many shapes and sizes. Under the influence of heat and in the presence of water, these granules swell and, eventually, disperse leading to a colloidal solution. Thus, the CWSS of the present invention will preferably have, before solubilisation, a granular structure similar to that of its corresponding native starch.

The CWSS of the present invention has a number average molecular weight (Mn) of 3 500 to 20 000 Daltons. Preferably, it will be between 5 000 and 15 000 Daltons.

The CWSS has a cold water solubility (SI) of 30-90%, preferably of 45-90%, more preferably of 50-80%. Cold water solubility is measured according to Method 1 set out below and generally refers to the proportion of starch granules that are able to swell in cold water (i.e. at neutral pH and at room temperature), forming a viscous, colloidal dispersion. Thus, cold water soluble starches may also be referred to as "cold water swellable" starches. As mentioned above, it is normally desirable for starches used in coating compositions to have very high levels of cold water solubility. It was therefore surprising to find that the CWSS of the present invention can be effective even at solubilities as low as 30%. Without wishing to be bound by theory, it is indeed believed that, despite being only slightly soluble under the standard conditions mentioned in Method 1, the CWSS of the present invention will fully disperse and solubilise when used in the preparation of a typical industrial coating composition, i.e. at a pH of 8-10 and at a temperature of 30-50°C. In any event, it should have a solubility (S2) at pH 10 / 35°C (see Method 2) which is at least 10% greater than (SI). Preferably, it will have a solubility (S2) of at least 50%. Even more preferably, it will have a solubility (S2) of at least 70%.

Coating compositions are typically used to enhance the feel, appearance and/or functionality of a substrate. As used in relation to the present invention, the term "coating composition" will refer to any aqueous solution or dispersion suitable for such a use, and to dry mixes used in their preparation. In the case of an aqueous solution or dispersion, it should ideally contain 30-75% dry substance by weight.

Preferably, the coating composition of the present invention will be a paper coating composition (also know as a "coating color"). It will advantageously comprise at least 50% dry substance by weight, more preferably 50-80%. The composition will advantageously have a pH of 7 to 12. Preferably, the pH will be from 8 to 10. In addition to the starchy material defined above, it will further contain one or more pigments. It may also contain one or more binders, one or more thickeners and one or more additives.

Examples of suitable pigments include: clays such as kaolin but also structured and calcined clays, hydrated aluminum silicates, bentonite, natural and synthetic calcium carbonate, calcium sulphate (gypsum), silicas, precipitated silicas, titanium dioxide, alumina, aluminium trihydrate, plastic (polystyrene) pigments, satin white, talc, barium sulphate, zinc oxide and mixtures of two or more thereof. The appropriate pigment will easily be selected by a skilled person depending on the type of coating composition to be obtained.

The composition of the invention may comprise: one or more binders. They can indeed be replaced, either in whole or in part, by the CWSS of the present invention. The binder can be selected - by way of example only - from carbohydrate- based binders including starch-based binders (such as oxidised or esterified starch) and cellulose binders (such as CMC and hydroxyethyl cellulose), protein binders (such as casein, gelatine, soy protein and animal glues) and synthetic binders, especially latex binders (such as styrene butadiene, styrene acrylate, vinyl polymer based latexes and polyvinyl alcohol) together with mixtures of two or more thereof.

The composition of the invention may comprise additional thickeners. Again, they can be replaced, in whole or in part, by the CWSS of the present invention. If further thickeners are used, they should not account for more than 50% of total thickener content on a dry weight basis. Examples of suitable thickeners include cellulose ethers (such as CMC, hydroxyethyl cellulose, hydroxypropyl cellulose, ethylhydroxyethyl cellulose and methyl cellulose), alginates (such as sodium alginate), xanthan, carrageenans, galactomannans (such as guar), native or modified starches (such as roll-dried starch), synthetic polymers (such as polyacrylates) and mixtures of two or more thereof.

The composition of the invention may comprise additives, if used, additives may include: surfactants (e.g. cationic surfactants, anionic surfactants, non-ionic surfactants, amphoteric surfactants and fluorinated surfactants), hardeners (e.g. active halogen compounds, vinylsulfone compounds, epoxy compounds, etc.), dispersing agents (e.g. polyacrylates, polyphosphates, polycarboxylates, etc.), flowability improvers, lubricants (e.g. calcium, ammonium and zinc stearate, wax or wax emulsions, alkyl ketene dimer, glycols, etc.), antifoamers (e.g. octyl alcohol, silicone-based antifoamers, etc.), releasing agents, foaming agents, penetrants, optical brighteners (e.g. fluorescent whiteners), preservatives (e.g. benzisothiazolone and isothiazolone compounds), biocides (e.g. metaborate, thiocyanate, sodium benzonate, etc.), yellowing inhibitors (e.g. sodium hydroxymethyl sulfonate, sodium p-toluenesulfonate, etc.), ultraviolet absorbers (e.g. benzotriazole compounds having a hydroxy-dialkylphenyl group at the 2 position), antioxidants (e.g. sterically hindered phenol compounds), insolubilisers, antistatic agents, pH regulators (e.g. sodium hydroxide, sulfuric acid, hydrochloric acid, etc.), water-resisting agents (e.g. ketone resin, anionic latex, glyoxal, etc.), wet and/or dry strengthening agents (e.g. glyoxal based resins, oxidised polyethylenes, melamine resins, urea formaldehyde, etc.), cross-linking agents, gloss-ink holdout additives.

### Example 1: Precoating of fine paper via Metered Size Press

### 1) Preparation of materials

| | Reference Precoat | Precoat of the invention |
|---|---|---|
| Coarse Ground Calcium Carbonate (parts) | 100 | 100 |
| Styrene Butadiene Latex (parts) | 6.5 | 5.5 |
| Chrono HV 117¹ (parts) | - | 3 |
| C*FilmTCF 07311 (parts) | 7 | 5 |
| Fluorescence Whitening Agent (parts) | 0.5 | 0.5 |
| Polyacrylate Thickener (parts) | 0.3 | 0.1 |
| Dry Solids (%) | 66.1 | 68.2 |

CWSS in accordance with the invention

| | Standard Middlecoat | Standard Topcoat |
|---|---|---|
| Ground Calcium Carbonate (parts) | 100 | 60 |
| Kaolin clay (parts) | - | 40 |
| Middlecoat latex (parts) | 5 | - |
| Topcoat Latex (parts) | - | 6.5 |
| C*FilmTCF 07311 (parts) | 7 | - |
| CMC (parts) | 0.3 | 0.35 |
| Fluorescence Whitening Agent (parts) | 0.1 | 0.2 |
| PVOH (parts) | - | 1 |
| Ca-stearate (parts) | - | 0.25 |
| Dry Solids (%) | 69 | 68.5 |

Reference precoat: the jet cooked (130°C) starch paste was added hot (> 80°C) into the pigments prior to the addition of latex and additives.

| | | |
|---|---|---|
| Top Latex 1 (parts) | 4.5 | 4 |
| Top Latex 2 (parts) | 1 | 1 |
| Chrono HV 170¹ (parts) | - | 2 |
| C*FilmTCF 07311 (parts) | 1 | - |
| Fluorescence Whitening Agent (parts) | 0.05 | 0.05 |
| PVOH (parts) | 0.3 | 0.3 |
| Polyacrylate Thickener (parts) | 0.5 | - |
| Dry Solids (%) | 70.3 | 71.8 |

CWSS in accordance with the invention

Reference topcoat: the jet cooked (130°C) starch paste was added hot (> 80°C) into the pigments prior to the addition of latex 1 and latex 2. Afterwards, the PVOH, FWA and thickener are added to the suspension.

Topcoat of the invention: Chrono HV 170 was mixed under high-shear conditions for 8 minutes in the pigment slurry/latex blend prior to the addition of PVOH and FWA.

2) Coating: 126 g/m² standard pre and middle coated paper used as base. 10.5 g/m² per side top-coat weight (stiff blade 0.508 mm, 1400 m/min). Paper was calendered at 200m/min, 80°C and at a nip pressure of 180kN/m.

The products were analysed using standard testing methods (the AA-GWR water release test, the Lehmann paper gloss 75° test, the Pfübau printing gloss test, the Pfübau mottling test and the coating cracking in the fold test). The results of these tests are shown in Figures 5 to 9. As can be seen, coating compositions according to the present invention lead to reduced water release, improved gloss (both paper and printing), less mottling and reduced cracking in the fold.

### Methods

### Method 1 - Cold Water Solubility (SI)

Determine the percent dry substance (DS) of the sample by drying 5g for 4 hours at 120°C under vacuum.

Precoat of the invention: Chrono HV 117 was mixed under high-shear conditions for 8 minutes in the pigment slurry/C*Film blend prior to the addition of latex, FWA and synthetic thickener.

2) Coating: 84 g/m² base paper with 10 g/m² per side pre-coat (MSP, 1000 m/min), followed by standard middle and top coats (free jet applicator, 1400 m/min). Paper was calendered at 200m/min, 80°C and at a nip pressure of 180kN/m.

The products were analysed using standard testing methods (the AA-GWR water release test, the Lehmann paper gloss 75° test, the Pfübau printing gloss test and the IGT pick-dry test). The results of these tests are shown in Figures 1 to 4. As can be seen, coating compositions according to the present invention lead to reduced water release, improved gloss (both paper and printing) and improved pick-dry properties.

### Example 2: Top coating of fine paper with free jet applicator

### 1) Preparation of materials

| | Standard Precoat | Standard Middlecoat |
|---|---|---|
| Coarse Ground Calcium Carbonate (parts) | 100 | 65 |
| Fine Ground Calcium Carbonate (parts) | - | 35 |
| Precoat latex (parts) | 6.5 | - |
| Middlecoat latex(parts) | - | 5 |
| C*Film TCF 07311 (parts) | 7 | 7 |
| CMC (parts) | - | 0.3 |
| Fluorescence Whitening Agent (parts) | 0.05 | 0.1 |
| Polyacrylate Thickener (parts) | 0.5 | - |
| Dry Solids (%) | 66.5 | 69 |

| | Reference Topcoat | Topcoat of the invention |
|---|---|---|
| Fine Ground Calcium Carbonate (parts) | 88 | 88 |
| Kaolin clay (parts) | 12 | 12 |
| Top Latex 1 (parts) | 4.5 | 4 |
| Top Latex 2 (parts) | 1 | 1 |
| Chrono HV 170¹ (parts) | - | 2 |
| C*Film TCF 07311 (parts) | 1 | - |
| Fluorescence Whitening Agent (parts) | 0.05 | 0.05 |
| PVOH (parts) | 0.3 | 0.3 |
| Polyacrylate Thickener (parts) | 0.5 | - |
| Dry Solids (%) | 70.3 | 71.8 |

| | | |
|---|---|---|
| ¹ Starchy material in accordance with the invention | | |

Reference topcoat: the jet cooked (130°C) starch paste was added hot (> 80°C) into the pigments prior to the addition of latex 1 and latex 2. Afterwards, the PVOH, FWA and thickener are added to the suspension.

Topcoat of the invention: Chrono HV 170 was mixed under high-shear conditions for 8 minutes in the pigment slurry/latex blend prior to the addition of PVOH and FWA.

2) Coating: 126 g/m² standard pre and middle coated paper used as base. 10.5 g/m² per side top-coat weight (stiff blade 0.508 mm, 1400 m/min). Paper was calendered at 200m/min, 80°C and at a nip pressure of 180kN/m.

The products were analysed using standard testing methods (the AA-GWR water release test, the Lehmann paper gloss 75° test, the Pfübau printing gloss test, the Pfübau mottling test and the coating cracking in the fold test). The results of these tests are shown in Figures 5 to 9. As can be seen, coating compositions according to the present invention lead to reduced water release, improved gloss (both paper and printing), less mottling and reduced cracking in the fold.

### Methods

### Method 1 - Cold Water Solubility (S1)

Determine the percent dry substance (DS) of the sample by drying 5g for 4 hours at 120°C under vacuum.

Weigh 2g of sample and transfer to a dry 200ml Kohlrausch flask. Partially fill with water at 25°C. Shake vigorously until completely in suspension and dilute to volume. Stopper flask and shake gently while submerged in a water bath at 25°C for a total agitation time of 1 hour.

Filter through a Whatman No. 2V paper, returning the first portion of filtrate. Measure 50ml of filtrate and transfer to a weighed evaporating dish.

Evaporate to dryness on a steam bath and dry in a vacuum oven for 1 hour at 100°C. Cool in a desiccator and weigh to the nearest mg. $DS , % = 100 - \left[\left(loss in weight, g \times 100\right) / \left(sample weight , g\right)\right]$ $Solubles, % = \left(residue weight, g \times 100\right) / \left[0.25 \times sample weight, g \times \left(DS , % / 100\right)\right]$

### Method 2 - Coating Colour Solubility (S2)

Determine the percent dry substance (DS) of the sample by drying 5g for 4 hours at 120°C under vacuum.

Weigh 2g of sample and transfer to a dry 200ml Kohlrausch flask. Partially fill with water at 35°C. Adjust pH with NaOH 0.1N until a pH value of 10.0 is reached. Shake vigorously until completely in suspension and dilute to volume. Stopper flask and shake gently while submerged in a water bath at 35°C for a total agitation time of 1 hour.

Filter through a Whatman No. 2V paper, returning the first portion of filtrate. Measure 50ml of filtrate and transfer to a weighed evaporating dish.

Evaporate to dryness on a steam bath and dry in a vacuum oven for 1 hour at 100°C. Cool in a desiccator and weigh to the nearest mg. $DS , % = 100 - \left[\left(loss in weight, g \times 100\right) / \left(sample weight , g\right)\right]$ $Solubles, % = \left(residue weight, g \times 100\right) / \left[0.25 \times sample weight, g \times \left(DS , % / 100\right)\right]$

### Method 3 - AA-GWR water release test

- ÅA - GWR WRV-apparatus
- Injection (10 mL)
- Thermometer
- Filter paper (blue ribbon)
- Millipore filter (5 µm pore size)
- Coating colour
- Stop-watch
- Balance (sensibility: 0,001g)

Both control levers - "Pressure" and "Cylinder" - have to be in the "off' position (downwards). At least three filter papers should be weighed and the figure logged (weight 1). The filters have to be placed on the rubberised plate and the Millipore filter is then placed on the filter papers with the shiny side up. Then the cylinder is placed on the plate with the ceiling upward. The whole composition is put on the metal plate and risen up by switching the "Cylinder" lever.

The sample is tempered to 30°C and 10 mL of the coating colour is filled into the cylinder with a syringe. The rubber should be free from coating colour to avoid leakage. The device has to be closed with the plug and the pressure is switched on with the "Pressure" lever and adjusted to 1 bar. At the same time the stop-watch is started. After two minutes, the pressure is stopped and the cylinder let down. The whole composition - plate, filters, cylinder - is removed and turned over a wash-basin and the filter paper is taken and weighed. This gives weight 2. Water retention is calculated as follows: WRV [g/m²] = (weight 2 - weight 1) * 1250

### Method 4 - Lehmann paper gloss 75° test

This test is performed according to Tappi T480 om-92.

### Method 5 - Prüfbau printing gloss test

Apparatus: Prüfbau apparatus
Printing ink: Lorilleux Rouge, Brilliant Standard 3810 (red)
Ink amount: 0.200cm³ for coated papers, 0.250cm³ for uncoated papers;
Time for ink distribution: 60 s
Time for inking: 30 s
Number of prints per inking: 3
Reinking: none
Pressure: 800 N
Speed: 1 m/s (constant)
Printing disc: Rubber 4 cm
Weighing unit: +/- 0.1 mg
Size of test stripe: width: 4.7 cm; length: 25 cm

The exact ink amount on the paper surface should be determined in [mg] or [g] by using an analytical balance (+/- 0.1 mg or +/- 0.0001 g exactly). The applied ink amount can be calculated by weighing the inked printing disc before and after printing.

Coat weight in [g/m²] = Coat weight in mg divided by 8 or Coat weight in g multiplied by 125 (printed area = 800 cm²)

3 stripes should be printed on each side. After drying the printed papers in a conditioned room (23°C/50%) for 24 hours the printing gloss should be determined either with Gardner or Lehmann glossmeter (10 measurements on each stripe). The printing gloss should be calculated to a coat weight of 1.2 g/m² for coated papers and 1.5 g/m² for uncoated papers by using regression analysis (either with calculator or Nomo-diagram).

### Method 6 - IGT pick-dry test

The dry-pick test is used to determine the surface strength of the coated and uncoated papers and boards. Picking is a surface damage caused by the adhesion force of the printing ink during the printing process. The adhesion force on the surface becomes higher at higher printing speeds and with inks exerting a higher tack. The printing pressure and ink layer thickness also influence the picking.
Test apparatus: IGT AIC2-5 apparatus
Testing ink: Lorilleux 3800-3806 depending on paper quality, IGT pick-oils with low, medium and high viscosities are also available.
Ink amount: 1.34 cm³ on the left inking cylinder and 0.94 cm³ on the right inking cylinder. 38 inking steps could be performed. 1 re-inking with 0.63 cm³ on the left cylinder: next 38 inking steps could be performed. After 1 re-inking the inking cylinders must be washed and started again.
Time of ink distribution: 2 x 60 s (re-inking 2 x 45 s)
Time for inking: 30 s on each inking cylinder
Pressure: 350 N /cm
Printing machine speed: accelerated speed depending on the paper surface strength Printing disc: Aluminium 1 cm
Blanket: paper
Size of test stripe: 2 cm ×30 cm

The printing disc is inked according to the IGT- procedure under above-mentioned conditions. At least 3 stripes of each sample and side are printed. Only the clear visible beginning of the picking is noticed. The pick result is calculated by means of the IGT-Nomogram.

**Viscosities of test inks for IGT dry pick:**

| **Ink type:** | **Viscosity at 23°C** |
|---|---|
| | **Pa.s** |
| H-oil | 110 |
| N-oil | 52 |
| L-oil | 17,5 |
| Lorilleux 3802 | 16 |
| Lorilleux 3803 | 26 |
| Lorilleux 3804 | 35 |
| Lorilleux 3805 | 40 |
| Lorilleux 3806 | 50 |

### Method 7 - Prüfbau mottling test

Mottling is the unevenness of the print of the paper or board due to irregular ink setting. It occurs on the multiple-colour offset machine by different film splitting on the successive rubber blankets and usually after first and second print. The mottling test simulates the printing process on the laboratory printing machine under constant conditions and evaluated visually after test printing.
Apparatus: Prüfbau apparatus
Printing ink: Blue ink type 520068 from M. Huber/Munich
Ink amount: 0.25 cm³
Time for ink distribution: 60 s
Time for inking: 30 s
Re-inking: none
Disc type: Rubber 4 cm for 1.print; Rubber 4 cm for 3 counter prints;
Pressure: 800 N for the printing disc; 800 N for 3 counter prints;
Speed: 0.5 m/sec (constant)
Time interval for the 3 counter prints: 1 s
Size of test stripe: width: 4.7 cm; length: 25 cm
Number of test: 1 stripe for each side

Test stripe should be printed under the above-mentioned conditions. Is after printing three counter prints must be done with the un-inked disc. The printed stripe is evaluated with an image analysing system via scanner.

The image of the paper strip is measured via a scanner in seven different resolution stages. The higher the calculated value, the stronger the mottling pronounced in this stage.

### Method 8 - Coating cracking in the fold test

Testing ink: Lorilleux Rouge Brilliant Standard 3810 (magenta)
Ink amount: 0.200 cm³
Time for ink distribution: 60 s
Time for inking: 30 s
Pressure: 800 N
Speed: 1 m/s (constant)
Printing disc: Rubber 4 cm
Balance: 0,1 mg exactly
Size of test stripe: width: 4.7 cm; length: 25 cm in machine direction

The exact ink amount on the paper surface should be determined in [mg] or [g] by using an analytical balance (+/- 0.1 mg or +/- 0.0001 g exactly). The applied ink amount can be calculated by weighing the inked printing disc before and after printing. Coat weight in [g/m²] = Coat weight in mg divided by 8 or coat weight in g multiplied by 125 (printed area=800cm²).

For each trial, 5 stripes are printed in machine direction. After conditioning the printed papers (23°C/50%) for 24 hours, each strip is laid separately in an oven for 15 seconds at 120 °C. With the printing side outside, the paper is slightly pre-folded and fixed on the Prüfbau rubber matrix.

Immediately afterwards, the paper was folded in the Prüfbau apparatus. The 5 strips were ranked and judged as a package.
Folding pressure: 1600 N
Folding (printing) disc: Aluminium 4 cm
Speed: 0,5 m/s (constant)

## Claims

1. A coating composition comprising a cold water soluble starch and one or more binders, thickeners and/or pigments **characterized in that** said cold water soluble starch is derived from a starch selected from the group consisting of wheat starch, corn starch and mixtures thereof, and has a DE of less than 5 and has:
- a number of average molecular weight (Mn) of 3500 to 20000 Daltons;
- a granular structure before solubilisation;
- a solubility at pH7 and 20°C (S1) of 30 to 90%; and
- a solubility at pH10 and 35°C (S2) which is at least 10% greater than S1.

2. The composition of claim 1, wherein S2 is greater than 50%.

3. The composition of claim 1, wherein S2 is greater than 70%.

4. The composition of claim 1, wherein the binder is selected from the group consisting of: styrene butadiene, styrene acrylate, vinyl polymer based latexes, polyvinyl alcohol, modified starches and mixtures of two or more thereof.

5. The composition of claim 1, wherein the thickener is selected from the group consisting of:
cellulose ethers, hydrocolloids, native or modified starches, synthetic polymers and mixtures of two or more thereof.

6. The composition of claim 1, wherein the pigment is selected from the group consisting of:
calcium carbonates, kaolin, talk, titanium dioxide, gypsum, engineered pigments, bentonite and mixtures of two or more thereof.

7. The composition of claim 1, further comprising one or more additives,

8. The composition of claim 7, wherein the one or more additives are selected from the group consisting of: dispersing agents, whitening agents, thickeners, rheology modifiers, cross-linking agents and biocides.

9. The composition of claim 1, wherein the pH of said composition is from 7 to 12.

10. The composition of claim 9, wherein the pH of said composition is from 8 to 10.

11. A paper coating composition according to claim 1.

12. The paper coating composition of claim 11, comprising at least 50% dry substance by weight.

13. The paper coating composition of claim 11, comprising 50-80% dry substance by weight.

14. The paper coating composition of claim 11, comprising 4-10% cold water soluble starch by weight dry substance.

15. A paper product coated with the coating composition of claim 1.

16. Use of a cold water soluble starch for the preparation of a coating composition **characterized in that** said cold water soluble starch is derived from a starch selected from the group consisting of wheat starch, corn starch and mixtures thereof, and has a DE of less than 5 and has:
- a number of average molecular weight (Mn) of 3500 to 20000 Daltons;
- a granular structure before solubilisation;
- a solubility at pH7 and 20°C (S1) of 30 to 90%; and
- a solubility at pH10 and 35°C (S2) which is at least 10% greater than S1.

## Patentansprüche

1. Beschichtungsgemisch, umfassend eine kaltwasserlösliche Stärke und eines oder eine Vielzahl von Bindemittel, Verdickungsmittel und/oder Pigmente, **dadurch gekennzeichnet, dass** die erwähnte kaltwasserlösliche Stärke von einer Stärke abgeleitet wird, die aus der Gruppe bestehend aus Weizenstärke, Maisstärke und deren Mischungen ausgewählt wird und eine DE von unter 5 sowie folgende Eigenschaften hat:
eine Anzahl von durchschnittlichem Molekulargewicht (Mn) von 3500 bis 20000 Dalton;
eine körnige Struktur vor der Solubilisierung;
eine Solubilität von 30 bis 90% bei pH7 und 20 °C (S1); und
eine Solubilität, die bei pH10 und 35 °C (S2) mindestens 10% höher ist als S1.

2. Gemisch nach Anspruch 1, wobei S2 höher als 50% ist.

3. Gemisch nach Anspruch 1, wobei S2 höher als 70% ist.

4. Gemisch nach Anspruch 1, wobei das Bindemittel aus der Gruppe bestehend aus Styrol-Butadien, Styrol-Acrylat, Vinylpolimer-basierten Latizes, Polyvinylalkohol, modifizierten Stärken und Mischungen aus zwei oder mehr davon ausgewählt wird.

5. Gemisch nach Anspruch 1, wobei das Verdickungsmittel aus der Gruppe bestehend aus Celluloseethern, Hydrokolloiden, natürlichen oder modifizierten Stärken, synthetischen Polymeren und Mischungen aus zwei oder mehr davon ausgewählt wird.

6. Gemisch nach Anspruch 1, wobei das Pigment aus der Gruppe bestehend aus Calciumcarbonaten, Kaolin, Talk, Titandioxid, Gips, veränderten Pigmenten, Bentonit und Mischungen aus zwei oder mehr davon ausgewählt wird.

7. Gemisch nach Anspruch 1, weiter umfassend einen oder eine Vielzahl von Zusatzstoffe.

8. Gemisch nach Anspruch 7, wobei der eine oder eine Vielzahl von Zusatzstoffe aus der Gruppe bestehend aus Dispergiermitteln, Weißmachern, Verdickungsmitteln, Rheologieadditiven, Vernetzungsmitteln und Bioziden ausgewählt werden.

9. Gemisch nach Anspruch 1, wobei der pH-Wert des erwähnten Gemisches in dem Bereich 7 bis 12 liegt.

10. Gemisch nach Anspruch 9, wobei der pH-Wert des erwähnten Gemisches in dem Bereich 8 bis 10 liegt.

11. Gemisch zu der Papierbeschichtung nach Anspruch 1.

12. Gemisch zu der Papierbeschichtung nach Anspruch 11, mit mindestens 50% Trockensubstanz nach Masse.

13. Gemisch zu der Papierbeschichtung nach Anspruch 11, mit 50-80% Trockensubstanz nach Masse.

14. Gemisch zu der Papierbeschichtung nach Anspruch 11, mit 4-10% kaltwasserlöslicher Stärke nach Masse Trockensubstanz.

15. Papierprodukt, beschichtet mit dem Beschichtungsgemisch nach Anspruch 1.

16. Verwendung einer kaltwasserlöslichen Stärke zu der Vorbereitung eines Beschichtungsgemisches, **dadurch gekennzeichnet, dass** die erwähnte kaltwasserlösliche Stärke von einer Stärke abgeleitet wird, die aus der Gruppe bestehend aus Weizenstärke, Maisstärke und deren Mischungen ausgewählt wird und eine DE von weniger als 5 sowie folgende Eigenschaften hat:
eine Anzahl von durchschnittlichem Molekulargewicht (Mn) von 3500 bis 20000 Dalton;
eine körnige Struktur vor der Solubilisierung;
eine Solubilität von 30 bis 90% bei pH7 und 20 °C (S1); und
eine Solubilität, die bei pH10 und 35 °C (S2) mindestens 10% höher ist als S1.

## Revendications

1. Composition de revêtement comprenant un amidon soluble dans l'eau froide et un ou plusieurs liants, épaississants et/ou pigments, **caractérisée en ce que** ledit amidon soluble dans l'eau froide est dérivé d'un amidon choisi dans le groupe constitué par l'amidon de blé, l'amidon de maïs et leurs mélanges, et présente une DE inférieure à 5 et présente :
- une masse moléculaire moyenne en nombre (Mn) de 3 500 à 20 000 Daltons ;
- une structure granulaire avant la solubilisation ;
- une solubilité à pH 7 et 20 °C (S1) de 30 à 90 % ; et
- une solubilité à pH 10 et 35 °C (S2) qui est supérieure d'au moins 10 % à S1.

2. Composition selon la revendication 1, dans laquelle S2 est supérieure à 50 %.

3. Composition selon la revendication 1, dans laquelle S2 est supérieure à 70 %.

4. Composition selon la revendication 1, dans laquelle le liant est choisi dans le groupe constitué par : le styrène butadiène, l'acrylate de styrène, les latex à base de polymère vinylique, l'alcool polyvinylique, les amidons modifiés et les mélanges de deux ou plusieurs d'entre eux.

5. Composition selon la revendication 1, dans laquelle l'épaississant est choisi dans le groupe constitué par : les éthers de cellulose, les hydrocolloïdes, les amidons natifs ou modifiés, les polymères synthétiques et les mélanges de deux ou plusieurs d'entre eux.

6. Composition selon la revendication 1, dans laquelle le pigment est choisi dans le groupe constitué par : les carbonates de calcium, le kaolin, le dioxyde de titane, le gypse, les pigments fabriqués, la bentonite et les mélanges de deux ou plusieurs d'entre eux.

7. Composition selon la revendication 1, comprenant en outre un ou plusieurs additifs.

8. Composition selon la revendication 7, dans laquelle le ou les additifs sont choisis dans le groupe constitué par : des agents dispersants, des agents blanchissant, des épaississants, des modificateurs de rhéologie, des agents de réticulation et des biocides.

9. Composition selon la revendication 1, dans laquelle le pH de ladite composition est de 7 à 12.

10. Composition selon la revendication 9, dans laquelle le pH de ladite composition est de 8 à 10.

11. Composition de revêtement de papier selon la revendication 1.

12. Composition de revêtement de papier selon la revendication 11, comprenant au moins 50 % en poids de substance sèche.

13. Composition de revêtement de papier selon la revendication 11, comprenant 50 à 80 % en poids de substance sèche.

14. Composition de revêtement de papier selon la revendication 11, comprenant de 4 à 10 % d'amidon soluble dans l'eau froide en poids de substance sèche.

15. Produit papier revêtu de la composition de revêtement de la revendication 1.

16. Utilisation d'un amidon soluble dans l'eau froide pour la préparation d'une composition de revêtement **caractérisée en ce que** ledit amidon soluble dans l'eau froide est dérivé d'un amidon choisi dans le groupe constitué par l'amidon de blé, l'amidon de maïs et leurs mélanges, et présente une DE inférieure à 5 et présente :
- une masse moléculaire moyenne en nombre (Mn) de 3 500 à 20 000 Daltons ;
- une structure granulaire avant la solubilisation ;
- une solubilité à pH 7 et 20 °C (S1) de 30 à 90 % ; et
- une solubilité à pH 10 et 35 °C (S2) qui est supérieure d'au moins 10 % à S1.
